



US009691544B2

(12) **United States Patent**  
**Sun**

(10) **Patent No.:** **US 9,691,544 B2**  
(45) **Date of Patent:** **Jun. 27, 2017**

(54) **ELECTROSTATICALLY TUNABLE MAGNETOELECTRIC INDUCTORS WITH LARGE INDUCTANCE TUNABILITY**

(75) Inventor: **Nian-Xiang Sun**, Winchester, MA (US)

(73) Assignee: **Winchester Technologies, LLC**,  
Winchester, MA (US)

(\*) Notice: Subject to any disclaimer, the term of this patent is extended or adjusted under 35 U.S.C. 154(b) by 207 days.

(21) Appl. No.: **14/241,032**

(22) PCT Filed: **Aug. 20, 2012**

(86) PCT No.: **PCT/US2012/051579**

§ 371 (c)(1),  
(2), (4) Date: **Feb. 25, 2014**

(87) PCT Pub. No.: **WO2013/026056**

PCT Pub. Date: **Feb. 21, 2013**

(65) **Prior Publication Data**

US 2014/0253272 A1 Sep. 11, 2014

**Related U.S. Application Data**

(60) Provisional application No. 61/524,913, filed on Aug. 18, 2011.

(51) **Int. Cl.**

**H01F 21/02** (2006.01)  
**H01F 5/00** (2006.01)

(Continued)

(52) **U.S. Cl.**

CPC ..... **H01F 29/146** (2013.01); **H01F 21/08** (2013.01); **H01F 41/046** (2013.01); **H01F 41/14** (2013.01);

(Continued)

(58) **Field of Classification Search**

CPC ..... H01F 21/08; H01F 41/046; H01F 41/045;  
H01F 21/06; H01L 41/044; H01L 2924/30107

(Continued)

(56) **References Cited**

**U.S. PATENT DOCUMENTS**

3,858,138 A 12/1974 Gittleman et al.  
6,037,649 A \* 3/2000 Liou ..... H01L 23/5227  
257/531

(Continued)

**OTHER PUBLICATIONS**

International Search Report & Written Opinion on PCT/US2012/051579 dated Nov. 2, 2012.

(Continued)

*Primary Examiner* — Alexander Talpalatski

*Assistant Examiner* — Joselito Baisa

(74) *Attorney, Agent, or Firm* — Foley & Lardner LLP;  
John D. Lanza

(57) **ABSTRACT**

An electrostatically tunable magnetoelectric inductor including: a substrate; a piezoelectric layer; and a magnetoelectric structure comprising a first electrically conductive layer, a magnetic film layer, a second electrically conductive layer, and recesses formed so as to create at least one electrically conductive coil around the magnetic film layer; with a portion of the substrate removed so as to enhance deformation of the piezoelectric layer. Also disclosed is a method of making the same. This inductor displays a tunable inductance range of >5:1 while consuming less than 0.5 mJ of power in the process of tuning, does not require continual current to maintain tuning, and does not require complex mechanical components such as actuators or switches.

**13 Claims, 4 Drawing Sheets**



|      |                                       |                                                                                        |                         |              |      |         |                           |
|------|---------------------------------------|----------------------------------------------------------------------------------------|-------------------------|--------------|------|---------|---------------------------|
| (51) | <b>Int. Cl.</b>                       |                                                                                        |                         |              |      |         |                           |
|      | <i>H01F 29/14</i>                     | (2006.01)                                                                              |                         | 7,800,278    | B2 * | 9/2010  | Ujihara .....             |
|      | <i>H01F 41/14</i>                     | (2006.01)                                                                              |                         |              |      |         | F03G 7/065<br>310/306     |
|      | <i>H01F 41/32</i>                     | (2006.01)                                                                              |                         | 8,134,444    | B2 * | 3/2012  | Horiuchi .....            |
|      | <i>H01F 21/08</i>                     | (2006.01)                                                                              |                         |              |      |         | H01F 17/0013<br>336/200   |
|      | <i>H01F 41/04</i>                     | (2006.01)                                                                              |                         | 8,143,987    | B2 * | 3/2012  | Kireev .....              |
|      | <i>H01F 10/26</i>                     | (2006.01)                                                                              |                         |              |      |         | H01L 23/5227<br>336/200   |
|      | <i>H01F 41/34</i>                     | (2006.01)                                                                              |                         | 8,797,711    | B2 * | 8/2014  | Matsumoto .....           |
| (52) | <b>U.S. Cl.</b>                       |                                                                                        |                         |              |      |         | H01G 4/30<br>361/303      |
|      | CPC .....                             | <i>H01F 41/32</i> (2013.01); <i>H01F 10/265</i> (2013.01); <i>H01F 41/34</i> (2013.01) |                         | 2002/0104990 | A1 * | 8/2002  | DeReus .....              |
| (58) | <b>Field of Classification Search</b> |                                                                                        |                         |              |      |         | B81B 3/0051<br>257/20     |
|      | USPC .....                            |                                                                                        | 336/30, 200             | 2003/0000058 | A1 * | 1/2003  | Tsai .....                |
|      |                                       | See application file for complete search history.                                      |                         |              |      |         | H03H 3/02<br>29/25.35     |
| (56) | <b>References Cited</b>               |                                                                                        |                         | 2003/0021004 | A1 * | 1/2003  | Cunningham .....          |
|      | U.S. PATENT DOCUMENTS                 |                                                                                        |                         |              |      |         | B81B 3/0051<br>359/290    |
|      | 6,065,353 A                           | 5/2000                                                                                 | Hirabayashi et al.      | 2005/0028336 | A1 * | 2/2005  | Robert .....              |
|      | 6,759,727 B2 *                        | 7/2004                                                                                 | Ju .....                |              |      |         | H03H 3/04<br>29/25.35     |
|      |                                       |                                                                                        | H01L 21/84<br>257/528   | 2006/0091608 | A1 * | 5/2006  | Yercha .....              |
|      | 7,144,101 B2 *                        | 12/2006                                                                                | Ifuku .....             |              |      |         | A63B 67/06<br>273/348.4   |
|      |                                       |                                                                                        | B41J 2/14233<br>347/72  | 2006/0256167 | A1   | 11/2006 | Ifuku et al.              |
|      | 7,146,861 B1 *                        | 12/2006                                                                                | Cook .....              |              |      |         | 2007/0045773              |
|      |                                       |                                                                                        | A61B 5/0215<br>73/715   |              |      |         | A1 .....                  |
|      | 7,170,384 B2 *                        | 1/2007                                                                                 | Kim .....               | 2008/0068759 | A1   | 3/2008  | Orlando et al.            |
|      |                                       |                                                                                        | H01F 17/0006<br>336/200 |              |      |         | 2008/0303624              |
|      | 7,250,831 B2 *                        | 7/2007                                                                                 | Song .....              |              |      |         | A1 .....                  |
|      |                                       |                                                                                        | H03H 3/02<br>216/17     | 2009/0189486 | A1 * | 12/2008 | Yamada et al.             |
|      | 7,262,680 B2 *                        | 8/2007                                                                                 | Wang .....              |              |      |         | 2009/0277300              |
|      |                                       |                                                                                        | H01F 17/0013<br>257/531 |              |      |         | A1 .....                  |
|      | 7,310,029 B2 *                        | 12/2007                                                                                | Robert .....            |              |      |         | H02N 2/025<br>310/323.02  |
|      |                                       |                                                                                        | H03H 3/04<br>310/312    |              |      |         | 74/99 R                   |
|      | 7,608,975 B2 *                        | 10/2009                                                                                | Orlando .....           | 2011/0128602 | A1 * | 6/2011  | Hamano .....              |
|      |                                       |                                                                                        | H01F 21/08<br>310/311   |              |      |         | G02B 13/0005<br>359/205.1 |
|      | 7,694,551 B2 *                        | 4/2010                                                                                 | Jakoby .....            | 2011/0205173 | A1 * | 8/2011  | Arai .....                |
|      |                                       |                                                                                        | G01N 11/16<br>73/54.26  |              |      |         | G06F 3/044<br>345/173     |
|      |                                       |                                                                                        |                         | 2011/0234351 | A1 * | 9/2011  | Kawarai .....             |
|      |                                       |                                                                                        |                         |              |      |         | H01F 21/06<br>336/30      |

## OTHER PUBLICATIONS

International Preliminary Report on Patentability on PCT/US2012/051579 dated Feb. 18, 2014.  
Chinese Office Action on 2012800511951 dated Nov. 3, 2015.

\* cited by examiner

FIG. 1



FIG. 2



**FIG. 3A****FIG. 3B**

FIG. 4

| Tunability - Material Combinations |                             |     |              |      |
|------------------------------------|-----------------------------|-----|--------------|------|
| Piezoelectric                      | PZT                         |     | PMN-PT       |      |
|                                    | $\Delta L/L$                | Q   | $\Delta L/L$ | Q    |
| MEMs Inductors                     | $\Delta L/L = 40\%$ , Q = 5 |     |              |      |
| Metglas                            | 900 %                       | 30  | 12000%       | 100  |
| Terfenol                           | 300%                        | 30  | 800%         | 100  |
| Galfenol                           | 1500%                       | 30  | 13000%       | 100  |
| Mn-Zn ferrite                      | 150%                        | ~50 | 2400%        | ~200 |

## 1

**ELECTROSTATICALLY TUNABLE  
MAGNETOELECTRIC INDUCTORS WITH  
LARGE INDUCTANCE TUNABILITY**

**CROSS REFERENCES TO RELATED  
APPLICATIONS**

This application claims the benefit of and priority under 35 U.S.C. §119(e) to U.S. Provisional Application No. 61/524,913, filed on Aug. 18, 2011, and entitled "Electrostatically Tunable Magnetoelectric Inductors With Large Inductance Tunability and Improved Performance," the disclosure of which is hereby incorporated herein by reference in its entirety.

**BACKGROUND**

The present disclosure relates generally to tunable magnetoelectric inductors with large inductance tunability and a method of manufacturing such inductors. The invention also relates to semiconductor devices containing tunable magnetoelectric inductors.

Incorporating tunability in conventional RF front-end components allows for the development of radio architectures capable of operating over multiple bands and standards, resulting in a reduction in cost, size, complexity, and power consumption of the radio transceiver. Front-end components such as tunable filters, phase shifters, voltage controlled oscillators, tunable low-noise amplifiers, and other RF components use on-chip and off-chip passive electronic components. Inductors, as one of the three fundamental components for electronic circuits, are extensively used in these front-end components as well as in other electronic applications. Tunable inductors, especially tunable inductors suitable for use in RF circuits, are key elements in creating intelligent, reconfigurable radios. While electronically tunable capacitors and resistors have been widely used for such tasks, electronically tunable inductors have not been readily available, despite the broad range of uses for such inductors.

Different technologies have been explored for tunable RF inductors, including inductors with magnetic materials where the permeability can be tuned by a magnetic field, inductors with magnetic materials where the permeability can be tuned by changing the coupling of the inductor coil and the magnetic core, inductors where the winding is digitally controlled via MEMS switches, mechanical tuning of mutual inductance between coupled inductors, varactor-based tunable inductors created by connecting a varactor with a fixed inductor so as to vary the bias voltage applied across the varactor and thus tuning the effective inductance, and manually tuned inductors. Each of these tunable inductor technologies has shortcomings that prevent general and widespread acceptance. Magnetic field tuning requires significant power and a constant current. Mechanical tuning requires large, complex actuators which are difficult to fabricate. Switchable inductors are limited by the number of switches used and the number of switches is limited as increasing this number reduces inductor quality. Varactor-tuned inductors have low quality factors and limited tunability. Manually tuned inductors are inconvenient to use. These negative aspects to currently available tunable inductors limit their usage.

**SUMMARY**

An electrostatically tunable inductor with a wide range of tunable inductance that does not require complex mechani-

## 2

cal actuators or switches and does not require significant consumption of power or an ongoing constant current draw is described.

In one or more embodiments, the electrostatically tunable inductor comprises a piezoelectric layer disposed above a substrate. Disposed above the piezoelectric layer is a magnetoelectric structure, comprising a first electrically conductive layer, a magnetic film layer adjacent to the first electrically conductive layer, and a second electrically conductive layer electrically connected to the first electrically conductive layer. A method of manufacture is also disclosed.

In one aspect, the electrostatically tunable inductor is manufactured by forming a piezoelectric layer disposed above a substrate. Disposed above the piezoelectric layer is a magnetoelectric structure, formed of a first electrically conductive layer, a magnetic film layer adjacent to the first electrically conductive layer, and a second electrically conductive layer electrically connected to the first electrically conductive layer.

The electrostatically tunable inductor is manufactured using techniques that are adapted from semiconductor manufacturing and allow the incorporation and/or integration of tunable inductor devices into semiconductor devices. In one or more embodiments, the tunable inductor is incorporated into the semiconductor device during the manufacture and assembly of the device.

**BRIEF DESCRIPTION OF THE DRAWINGS**

The above and other objects and advantages of the present invention will be apparent upon consideration of the following detailed description, taken in conjunction with the accompanying drawings, in which like reference characters refer to like parts throughout, and in which:

FIG. 1 is a schematic illustration of an electrostatic tunable inductor according to one or more embodiments;

FIGS. 2A-2F are process cross-sectional views illustrating an electrostatically tunable magnetoelectric inductor and a method for manufacturing such a device according to certain embodiments.

FIGS. 3A-3B are schematics of a multilayer magnetic/piezoelectric material showing the mechanism by which an electric field induces a magnetic field;

FIG. 4 is a table of tunability and quality factors of the tunable magnetoelectric inductor of FIG. 1 using different magnetic and piezoelectric materials, in accordance with certain embodiments.

**DETAILED DESCRIPTION OF THE  
INVENTION**

The present disclosure provides for tunable magnetoelectric inductors with large inductance tunability and improved performance over the prior art. Additionally, the present disclosure provides for a method of manufacturing such an inductor suitable for integration into standard semiconductor manufacturing processes. Unlike other tunable inductors, the electrostatically tunable magnetoelectric inductor of this disclosure displays a tunable inductance range of >5:1 while consuming less than 0.5 mJ of power in the process of tuning, does not require continual current to maintain tuning, and does not require complex mechanical components such as actuators or switches.

A magnetoelectric inductor 200 according to one or more embodiments is described with reference to FIG. 1. In certain embodiments the magnetoelectric inductor includes

a substrate 202 such as silicon, sapphire, or such other substrates as may be used in semiconductor manufacturing processes. The inductor includes a piezoelectric layer 204, composed of a piezoelectric material. A first isolation layer 206 composed of an isolation material such as silicon dioxide or other conventional dielectric material is deposited over the piezoelectric material. The isolation layer separates the piezoelectric material from the magnetoelectric structure, but provides a means for translating the changes in strain from the piezoelectric layer to the magnetic structure. A magnetoelectric structure, such as a magnetic solenoid or toroid inductor, is arranged above the piezoelectric layer. The magnetoelectric structure includes conductive metal layers 208a, 208b such as copper, aluminum, silver or other conductive metal which are deposited above and below a high permeability magnetic film 210 to form a solenoid coil. A solenoid is a magnetic field coil which produces a fairly uniform magnetic field in its interior. Like all current carrying devices, it has inductance in proportion to the volume integral of the square of the magnetic field for a give current. Solenoids are typically formed by helically winding a conductive wire into a coil. In the current embodiment, the solenoid coil is formed by joining patterned upper and lower conductive layer using vias 212a, 212b to provide a coiled conductive pathway around the magnetic film layer.

After deposition, the magnetic film is magnetically annealed to align magnetic domains and patterned to enhance the permeability of the material. In one or more embodiments, each of the layers in the magnetoelectric inductor are spaced apart from one another by an isolation layer. This structure leads to enhanced tunable inductance range and quality factor over previous tunable inductors integrated into semiconductor devices.

FIG. 2F is a schematic of an electrostatically tunable magnetoelectric inductor 100 in accordance with certain embodiments. The inductor 100 includes a substrate layer 101 and a piezoelectric layer 102 above substrate layer 101. A first isolation layer 103 is above the piezoelectric layer 102. A first electrically conducting layer 104 is above the first isolation layer 103. In some embodiments, the first electrically conducting layer is patterned. A magnetic film layer 105 is above the first electrically conducting layer 104. In some embodiments, the magnetic film layer 105 is annealed to align magnetic domains and patterned. In some embodiments, the patterning is performed by etching. A second isolation layer 106 is above the magnetic film layer 105 and the first electrically conducting layer 104.

In some embodiments, recesses 107 are formed in the second isolation layer. The recesses 107 are formed so as to penetrate the second isolation layer 106 and expose a surface of the first electrically conducting layer 104. While two recesses 107 are shown in device 100, any number of recesses may be used for a particular device (e.g., 1, 3, etc.). A second electrically conducting layer 108 is above at least part of the second isolation layer 106, and is so placed as to fill the at least one recess 107 and contact the first electrically conducting layer 104. In some embodiments, the second electrically conducting layer 108 is patterned. In some embodiments, the patterning of the first electrically conducting layer 104 and the second electrically conducting layer 108 are arranged, in combination with the arrangement of the recesses 107, so as to form at least one coil around the magnetic film layer 109. In some embodiments, a portion of the substrate 101 below the piezoelectric layer is thinner than the portion of the substrate not below the piezoelectric layer 109 in order to maximize the deformation of the piezoelectric layer for a given induced electric field.

Further, the configurations shown in FIG. 1 and FIG. 2F are intended to be exemplary and is not intended to be limiting. One of skill can appreciate that other variations of electrostatically tunable magnetoelectric inductors can be engineered according to the principles described herein without departing from the spirit of the description. Further, one of skill can appreciate that other electrostatically tunable magnetoelectric devices than inductors can be engineered according to the principles described herein without departing from the spirit of the description.

In some embodiments, the substrate layer 101 is composed of silicon. In other embodiments, it may be composed of gallium arsenide, gallium nitride, sapphire, or another substrate material. In some embodiments, the piezoelectric layer 102 is a layer of lead zirconate titanate (PZT) of about 1 to 20  $\mu\text{m}$  thickness, placed on the substrate. Doping of these lead zirconate-titanate ceramics (PZT) with, for example, Ni, Bi, Sb, Nb ions etc., make it possible to adjust individual piezoelectric and dielectric parameters as required. Other exemplary piezoelectric materials include PMN-PT (lead manganese niobate-lead titanate), PZN-PT (lead zinc niobate-lead titanate),  $\text{BaTiO}_3$ ,  $(\text{Ba},\text{Sr})\text{TiO}_3$ ,  $\text{ZnO}$ , and  $\text{AlN}$ . In some embodiments, the layer of lead zirconate titanate is composed of lead zirconate titanate with a ratio of about 52 parts zircon to 48 parts titanium. In other embodiments, the piezoelectric layer 102 is a layer of lead magnesium niobate-lead titanate. In some embodiments, the layer of lead magnesium niobate-lead titanate is composed of lead magnesium niobate-lead titanate with a ratio of about 65 parts lead magnesium niobate to 35 parts lead titanate. In some embodiments, the layer of lead zirconate titanate is of a thickness of about 5 to 10  $\mu\text{m}$ . In some embodiments, the first isolation layer 103 and second isolation layer 106 are composed of silicon dioxide. In some embodiments, the first electrically conducting layer 104 and second electrically conducting layer 108 are composed of copper. Exemplary magnetic materials or magnetic/non-magnetic insulator multilayers include those having high permeability, low loss tangent, and high resistivity. In some embodiments, the magnetic film layer 105 is composed of Metglas 2605CO<sup>TM</sup>. In other embodiments, the magnetic film layer 105 is composed of galfenol, terfenol, CoFeB, CoFeN, CoFe, or ferrites with a thickness based on the inductance required and the magnetoelectric strain change of the material.

A method of manufacturing an electrostatically tunable magnetoelectric inductor with large inductance tunability is also disclosed. As shown in FIG. 2A, a piezoelectric layer 102 is formed on a substrate 101. After the piezoelectric layer 102 is formed, a first isolation layer 103 is formed on the piezoelectric layer 102. In some embodiments, the piezoelectric layer 102 and first isolation layer 103 are formed by chemical vapor deposition. As shown in FIG. 2B, after the first isolation layer 103 is formed, a first electrically conducting layer 104 is formed on the first isolation layer 103. In some embodiments, the first electrically conducting layer is formed by sputtering of a copper seed layer, followed by application of photoresist and electrodeposition of a copper layer. In some embodiments, the photoresist is patterned so as to deposit the first electrically conducting layer in a pattern.

Then, as shown in FIG. 2C, a magnetic film layer 105 is formed on the first electrically conducting layer 104. In some embodiments, the magnetic film layer is formed by sputtering. In some embodiments, the magnetic film layer 105 is annealed after it is formed to align the magnetic domains within the magnetic film layer 105. Annealing increases the permeability of the magnetic film layer. In

some embodiments, the magnetic film layer 105 is patterned. In some embodiments, patterning of the magnetic film layer 105 into different geometries such as long stripe structures either along the length or width direction is achieved by etching. Patterning is used for adjustment of the magnetic anisotropy and achieving appropriate inductance and operation frequency. As shown in FIG. 2D, after deposition and optional annealing and patterning of the magnetic film layer 105, a second isolation layer 106 is formed on the magnetic film layer 105. In some embodiments, the second isolation layer 106 is deposited via chemical vapor deposition.

In some embodiments, as shown in FIG. 2D, recesses 107 are then formed on the second isolation layer 106. The recesses 107 are formed so as to penetrate the second isolation layer 106 and expose a main surface of the first electrically conducting layer 104 at a bottom portion of the recess 107. In some embodiments these recesses are formed via application of masked photoresist and etching of the second isolation layer 106. In some embodiments the mask used to apply photoresist is patterned. In some embodiments the photoresist mask pattern is so disposed as to form vias through which the first and second layer may be in electrical communication with one another. In further embodiments, the photoresist mask pattern is so disposed, in conjunction with the patterning of the first and second electrically conductive layers, as to arrange the vias and the electrically conductive layers in at least one coil formed around the magnetic film layer. In some embodiments, as shown in FIG. 2E, a second electrically conducting layer 108 is formed to cover at least part of the second isolation layer. In some embodiments, the second electrically conducting layer 108 is formed by sputtering of a copper seed layer, followed by application of photoresist and electrodeposition of a copper layer. In some embodiments, the photoresist is patterned so as to deposit the second electrically conducting layer 108 in a pattern. In some embodiments, as shown in FIG. 2F, the substrate 101 is removed below the magnetic film layer 105. In some embodiments, the substrate 101 is removed by etching of the substrate 101. Removal of the substrate 101 below the piezoelectric layer 102 helps to enhance deformation of the piezoelectric layer 102, thus increasing deformation of the magnetic film layer 105. By increasing this deformation, the change in permeability of the magnetic film layer 105 is increased and tunability of the completed electrostatically tunable magnetoelectric inductor 100 is enhanced.

As shown in FIGS. 3A-3B, induction of an electric field in the piezoelectric layer 301 can induce a magnetic field in the magnetic film layer 302. FIG. 3A shows the magnetic film device prior to induction of an electric field, with piezoelectric layer 301 and magnetic film layer 302 not deformed. Without an electric field applied, the inductance of the inductor rolls off quickly at higher frequencies (>10 kHz). This roll off is associated with the large eddy current loss in the magnetic film layer, leading to reduced effective permeability at high frequencies and thus lower inductance. As shown in FIG. 3B, when an electric field 303 is applied along the thickness direction of the piezoelectric layer 301, the piezoelectric layer 301 will deform in plane of the piezoelectric layer 301. This deformation will be transferred to the magnetic film layer 302, either directly or through intervening layers, inducing anisotropic magnetic fields 304 due to the inverse magnetoelectric effect. The anisotropy can be expressed by the following equation:

$$H_{eff} = H_a + H_{ME} = H_a + \frac{3\lambda_s Y d_{31} E}{M_s} \quad (1)$$

where  $H_a$  is the intrinsic anisotropy,  $H_{ME}$  is the induced anisotropy field due to magnetoelectric coupling,  $\lambda_s$  is the saturation magnetostriction constant,  $Y$  is the Young's modulus,  $d_{31}$  is the piezoelectric coefficient of the piezoelectric layer,  $E$  is the electric field across the piezoelectric layer, and  $M_s$  is the saturation magnetization of the magnetic layer. The converse magnetoelectric coupling coefficient is thus expressed by the following equation:

$$\alpha_{ME} = \frac{3\lambda_s Y d_{31}}{M_s} \quad (2)$$

From the effective magnetic anisotropy, the effective relative permeability of the magnetic film layer can be expressed as:

$$\mu_r = \frac{4\pi M_s}{H_{eff}} + 1 \quad (3)$$

and the inductance can be calculated as:

$$L = \mu_0 \frac{2\mu_r t + d}{d} \frac{N^2 A}{l} \quad (4)$$

where  $N$  is the number of turns of coil around the magnetic film layer,  $A$  is the cross-sectional area of the coil around the magnetic film layer,  $l$  is the length of the coil around the magnetic film layer,  $t$  is the thickness of the magnetic film layer, and  $d$  is the height of the magnetic film layer. Because effective magnetic anisotropy varies with induced electric field across the piezoelectric, effective relative permeability varies with effective magnetic anisotropy, and inductance varies with effective relative permeability, application of an electric field across the piezoelectric layer produces variation in inductance, enabling tunability of the magnetoelectric inductor. A strong electric field dependence of the inductance can be observed, with inductance decreasing rapidly at higher electric fields.

A high converse magnetoelectric coupling coefficient is desirable for achieving large tunability in tunable magnetoelectric inductors. Piezoelectric materials with a high piezoelectric coefficient and magnetic materials with a high saturation magnetostriction constant and low saturation magnetization are desirable to achieve a stronger converse magnetoelectric coupling coefficient and thus a greater tunable inductance range. It is also desirable that the magnetic material have a low loss tangent in order to improve the quality factor  $Q$  of the tunable inductor. Quality factor also varies with application of electric field, as the reduced permeability achieved at higher electric fields leads to increased skin depth and reduced core eddy current loss in combination with the increased peak quality factor frequency, also due to reduced permeability. At lower frequencies, inductance tunability is much greater as eddy current loss is not significant.

Tuning of the electrostatically tunable magnetoelectric inductor 100 is thus accomplished by deformation of the piezoelectric layer 102 via an electric field across the piezo-

electric layer. Deformation of the piezoelectric layer **102** induces a deformation of the magnetic film layer **105**. Deformation of the magnetic film layer **105** then leads to an effective magnetic anisotropy field due to the inverse magnetoelastic effect. This anisotropy field leads to a change in relative permeability of the magnetic film layer **105** and thus to a change in inductance **L** of the electrostatically tunable magnetoelectric inductor **100** as per equations 1-4 above. The inductance **L** of the electrostatically tunable magnetoelectric inductor **100** varies as per equation 4 above directly as a function of the relative permeability of the magnetic film layer **105**, which can be calculated by equation 3, where  $M_s$  is the saturation magnetization of the magnetic film layer **105** and  $H_{eff}$  is the total effective anisotropy field in the magnetic film layer **105**. Thus inducing deformation of the piezoelectric layer **102** leads to tuning of the inductance of the electrostatically tunable magnetoelectric inductor **100**. A tunable inductance range of >5:1 with low power consumption is achieved.

Deformation of the piezoelectric layer **102** within the device is advantageously achieved by taking advantage of the capacitive properties of the piezoelectric layer **102**. An applied voltage across the piezoelectric layer **102** can lead to a piezoelectric strain, which leads to a strain in the magnetic material, and therefore a change of the permeability. The electrical energy required to induce an applied voltage can be estimated from the energy associated with charging a piezoelectric capacitor, expressed as  $E = \frac{1}{2}CV^2$ , where  $C$  is the capacitance associated with the piezoelectric layer and  $V$  is the voltage to be induced across the piezoelectric layer. The stored electrical energy induces a voltage across the thickness of the piezoelectric layer **102** corresponding to an electric field across the piezoelectric layer **102** dependent on the thickness of the piezoelectric layer **102** and the voltage. The induced electric field deforms the piezoelectric layer **102** via the piezoelectric effect. By varying the stored charge, the induced electric field varies, which in turn varies the relative permeability. Variation of relative permeability allows tuning of inductance. As charge leakage from the piezoelectric layer **102** can be made negligibly small, tuning does not require the continual induction of an electric field but rather can be accomplished by one time induction of a charge across the piezoelectric layer.

Upon review of the description and embodiments of the present invention, those skilled in the art will understand that modifications and equivalent substitutions may be performed in carrying out the invention without departing from the essence of the invention. Thus, the invention is not meant to be limiting by the embodiments described explicitly above, and is limited only by the claims which follow.

What is claimed is:

1. An electrostatically tunable magnetoelectric inductor device comprising:  
a substrate;  
a piezoelectric layer disposed above the substrate;  
a magnetoelectric structure disposed above the piezoelectric layer comprising:  
a magnetic film layer experiencing deformation when the piezoelectric layer is deformed;  
an isolation layer disposed between the magnetic film layer and the piezoelectric layer, translating changes in strain from the piezoelectric layer to the magnetic film layer;  
a first electrically conductive layer and a second electrically conductive layer disposed on opposing sides of the magnetic film layer and in electrical communication with one another through at least one via defined by the isolation layer so as to form at least one electrically conductive coil around the magnetic film layer.
2. The device of claim 1, wherein the first electrically conductive layer is directly adjacent to the magnetic film layer.
3. The device of claim 1, wherein the magnetic film layer comprises an annealed magnetic film.
4. The device of claim 1, wherein the magnetic film layer is patterned.
5. The device of claim 1, wherein the substrate is thinner below the magnetic film device.
6. The device of claim 1, wherein the magnetic film layer is composed of a multilayer magnetic material.
7. The device of claim 1, wherein the first electrically conducting layer is composed of copper.
8. The device of claim 1, wherein the second electrically conducting layer is composed of copper.
9. The device of claim 1, wherein the piezoelectric layer has a composition represented by the formula  $PbZr_xTi_{1-x}O_3$ , wherein  $x$  satisfies  $0 < x < 1$ .
10. The device of claim 9, wherein  $x$  is within the range of 0.50 to 0.54.
11. The device of claim 1, wherein the piezoelectric layer has a composition represented by the formula  $(1-y)Pb(Mg_{1/3}Nb_{2/3})O_3 - y PbTiO_3$ , wherein  $y$  satisfies  $0 \leq y < 1$ .
12. The device of claim 11, wherein  $y$  is within the range of 0.32-0.38.
13. The device of claim 12, wherein the magnetic film layer is composed of a material selected from the group consisting of Metglas™, terfenol, galfenol, or manganese-zinc ferrite.

\* \* \* \* \*